

Patented June 27, 1939

2,163,820

# UNITED STATES PATENT OFFICE

2,163,820

## PHOTOGRAPHIC DEVELOPER

Gustav Wilmanns, Wolfen, Bitterfeld, and Wilhelm Schneider and Alfred Fröhlich, Dessau Anhalt, Germany, assignors, by mesne assignments, to Agfa Ansco Corporation, Binghamton, N. Y., a corporation of Delaware

No Drawing. Application March 19, 1937, Serial No. 131,780. In Germany April 23, 1936

12 Claims. (Cl. 95—88)

Our present invention relates to a process of developing photographic silver halide emulsions and more particularly to a process in which the developing agent used is a derivative of an organic 5 diamine, one amino-group of said diamine carrying a ring member, such as for instance



10 said ring member forming a hydrogenized ring together with the carbon-atom in ortho-position of the substituted amino-group or with the other amino-group.

An object of our invention is the new developing 15 process and a further object of our invention is the provision of the new developing preparations containing said derivatives of benzene diamines. Another object of our invention relates to developing colored pictures with the aid of said 20 compounds.

The invention is based on the observation that such diamines of the benzene series are valuable developing agents in which at least one amino-group is a member of a hydrogenized nucleus and the second amino-group is in such a position to 25 the other that formation of quinonoid compounds becomes possible. In other words we may use for instance tetrahydroquinoxaline:



5-amino-2-methylindole



6-amino-8-methoxy-1,2,3,4-tetrahydroquinoline



6-amino-8-methoxy-1,2,3,4-tetrahydroquinaldine



5-aminobenzothiazoline



60 and substitution products thereof. These od-

ucts develop the latent silver image in presence of alkali with or without a sulfite more powerfully than the known para-phenylenediamine and produce a very fine grain. For the purpose of obtaining special gradation the substances may be used in intermixture with each other or with a known developer. In combination with substances suitable for color development such as for instance phenyl-methyl-pyrazolone,  $\alpha$ -hydroxy-naphthoic acid, phenyl-isoxazolone and the chloranilide of benzoyl acetic ester, they are also useful particularly when the amino-group is in the para-position to the nuclear amino-group for the color development of single layer or multi-layer photographic material.

15 The following examples illustrate developers suitable for the invention:

### Example 1

A developer suitable for very fine grain work 20 consists of the following solution:

|                           |                   |      |
|---------------------------|-------------------|------|
| Water                     | cubic centimeters | 100  |
| Tetrahydroquinoxaline     | grams             | 1.5  |
| Calcined sodium carbonate | do                | 3    |
| Anhydrous sodium sulfite  | do                | 3 25 |

### Example 2

|                                                 |                   |      |
|-------------------------------------------------|-------------------|------|
| Water                                           | cubic centimeters | 100  |
| 6-amino-8-methoxy-1,2,3,4-tetrahydroquinoxaline | gram              | 1 30 |
| Calcined sodium carbonate                       | grams             | 3    |
| Anhydrous sodium sulfite                        | do                | 3    |

### Example 3

|                                                 |                   |     |
|-------------------------------------------------|-------------------|-----|
| Water                                           | cubic centimeters | 100 |
| 6-amino-8-methoxy-1,2,3,4-tetrahydroquinoxaline | gram              | 1   |
| Calcined sodium carbonate                       | grams             | 3   |
| 1-phenyl-3-methyl-5-pyrazolone                  | gram              | 0.5 |

### Example 4

|                                |                   |      |
|--------------------------------|-------------------|------|
| Water                          | cubic centimeters | 100  |
| 5-amino-dihydro-2-methylindole | gram              | 1    |
| Calcined sodium carbonate      | grams             | 3    |
| Anhydrous sodium sulfite       | do                | 3 45 |

### Example 5

|                           |                   |      |
|---------------------------|-------------------|------|
| Water                     | cubic centimeters | 100  |
| Calcined sodium carbonate | grams             | 3    |
| 5-aminobenzothiazoline    | gram              | 1 50 |

The developer according to Example 3 produces in addition to the silver image a dyestuff image in blue-red, from which by means of a suitable bath ("Farmer's reducer") the silver image may be removed so that a pure colored image remains.

55 By using other components instead of the 1-phenyl-3-methyl-5-pyrazolone other colored images may be obtained. Our invention is not limited to the examples given, but we contemplate as included all such modifications and equivalents

as fall within the scope of the appended claims. Needless to say that our new developers may be used in combination with any of the already known developers and the compounds producing a colored image together with the new developers are not limited to the examples given in our specification.

By introducing the coupling component into the individual layers of a multi-layer material a 3-10 color image can be produced by development either by the negative process or by the reversal process, the image being in complementary colors in the first case and in correct colors in the second case.

15 The methylene group or groups concerned in the ring formation may carry substituents which may be of a character suitable for lending solubility to the developer, such as for instance the hydroxy group and hydroxy-ethyl group.

20 What we claim is:

1. A process of developing photographic silver halide emulsions which comprises treating the said material in an aqueous solution of tetrahydro-quinoxaline sodium carbonate and sodium sulfite.

25 2. A process of developing photographic silver halide emulsions which comprises treating the said material in an aqueous solution of 6-amino-8-methoxy-1,2,3,4-tetrahydroquinoline, sodium carbonate and sodium sulfite.

30 3. A process of developing photographic silver halide emulsions which comprises treating the said material in an aqueous solution of 6-amino-8-methoxy-1,2,3,4-tetrahydroquinaldine, sodium carbonate and 1-phenyl-3-methyl-pyrazolone.

4. As a composition of matter, a photographic developer containing tetrahydroquinoxaline sodium carbonate and sodium sulfite.

5. As a composition of matter, a photographic developer containing 6-amino-8-methoxy-1,2,3,4-tetrahydroquinoline sodium carbonate and sodium sulfite.

6. As a composition of matter, a photographic developer containing 6-amino-8-methoxy-1,2,3,4-tetrahydroquinaldine sodium carbonate and 1-phenyl-3-methyl-pyrazolone.

7. A process of developing photographic silver halide emulsions, which comprises treating said emulsions in a bath containing a heterocyclic diamine of the benzene series hydrogenized in the heterocyclic nucleus selected from the group consisting of 5-aminodihydroindoles, 6-aminotetrahydroquinolines, 5-aminobenzothiazolines, tetrahydroquinoxalines, and alkyl- and oxalkyl substitution products thereof.

8. As a composition of matter a photographic developer containing an alkali metal sulfite, an alkali metal carbonate and a heterocyclic diamine of the benzene series hydrogenized in the heterocyclic nucleus, said diamine being selected from the group consisting of 5-aminodihydroindoles, 6-aminotetrahydroquinolines, 5-aminobenzothiazolines, tetrahydroquinoxalines, and alkyl- and oxalkyl substitution products thereof.

9. As a composition of matter a photographic developer for color forming development containing an alkali metal sulfite, an alkali metal carbonate and a diamine of the benzene series corresponding to the following general formula



wherein

Y is selected from the group consisting of  $-\text{CH}_2-\text{CH}_2$ ,  $-\text{CH}_2-\text{S}$ ;

Z is a member of the group consisting of H,  $-\text{OCH}_3$ ;

R1 is a member of the group consisting of  $-\text{CH}_3$ , H,  $-\text{CH}_2\text{CH}_2\text{OH}$ ;

said developer being capable of forming a dyestuff with a dyestuff component for color forming development.

10. A process of developing silver halide emulsions, which comprises treating said material in a bath containing a diamine of the benzene series corresponding to the following general formula 15



wherein

Y is a member of the group consisting of  $\text{CH}_2-\text{CH}_2$ ,  $\text{CH}_2-\text{S}$ ;

Z is a member of the group consisting of H,  $-\text{OCH}_3$  and  $\text{CH}_3$ ;

R1 is a member of the group consisting of  $\text{CH}_3$ , H,  $-\text{CH}_2\text{CH}_2\text{OH}$ .

30 11. A process of developing silver halide emulsions, which comprises treating said material in a bath containing a diamine of the benzene series corresponding to the following general formula



40 wherein

Y is a member of the group consisting of  $\text{CH}_2-\text{CH}_2$ ,  $\text{CH}_2-\text{S}$ ;

Z is a member of the group consisting of H,  $-\text{OCH}_3$  and  $\text{CH}_3$ ;

R1 is a member of the group consisting of  $\text{CH}_3$ , H,  $-\text{CH}_2\text{CH}_2\text{OH}$ ;

said diamine being used in combination with a dyestuff component for color forming development.

50 12. As a composition of matter a photographic developer comprising an alkali metal sulfite, an alkali metal carbonate and a compound corresponding to the following general formula



60 wherein

Y is a member of the group consisting of  $\text{CH}_2-\text{CH}_2$ ,  $\text{CH}_2-\text{S}$ ;

Z is a member of the group consisting of H,  $-\text{OCH}_3$  and  $\text{CH}_3$ ;

R1 is a member of the group consisting of  $\text{CH}_3$ , H,  $-\text{CH}_2\text{CH}_2\text{OH}$ .

70 GUSTAV WILMANNS.  
WILHELM SCHNEIDER.  
ALFRED FRÖHLICH.